

Dec. 25, 1928.

1,696,395

E. GATHMANN

SHRINK HEAD CASING FOR INGOT MOLDS

Filed Oct. 28, 1926



*Inventor:*  
*Emil Gathmann*  
*by his Attorneys*  
*Frederick Wight*

Patented Dec. 25, 1928.

1,696,395

# UNITED STATES PATENT OFFICE.

EMIL GATHMANN, OF BALTIMORE, MARYLAND.

## SHRINK-HEAD CASING FOR INGOT MOLDS.

Application filed October 28, 1926. Serial No. 144,800.

This invention relates to what are known as feeders, hot tops, or shrink head casings for ingot molds, in which provision is made for conserving the heat of the molten metal 5 in the top portion of the mold, in order that such portion of the metal may be maintained in a liquid condition, and thus serve to fill the pipe or cavity in the upper part of the body of the ingot, and thus reduce 10 the unsound or pipe-containing portion of the ingot in the top of the mold.

Such shrink head casings have usually been made of refractory material such as fire clay, and it has heretofore been proposed to construct feeders with chambers for containing combustible material such as coal, charcoal, or coke which, when burned, serves to conserve the heat of the ingot to some extent, and to thus reduce pipe. It has 20 also been heretofore proposed to make shrink head casings of combustible material such as coal, charcoal, coke or the like, and I therefore do not claim as my invention such subject matter.

According to my present invention, I construct a shrink head casing by forming the body thereof of slowly combustible material such as coke or coal or charcoal and a suitable binder such as Portland cement, 30 and I surround this casing with a non-combustible material preferably composed of silica sand, cement, and a small percentage of molasses. This non-combustible material is so applied as to form a sheath or casing 35 for the combustible material, which is closed at all points except at the top, where it is provided with a few or a plurality of openings which serve as vent holes.

Such shrink head casing may be made in 40 various shapes and sizes. Preferably the body of the shrink head casing is first molded and then dipped into a bath composed of silica sand, water, cement, and molasses in such manner as to apply the required 45 amount of such material to the core, and then the vent holes may be formed by drilling, or in other suitable way.

The accompanying drawing shows a vertical section of the upper part of an ingot 50 mold and a vertical section of a shrink head casing applied thereto constructed in accordance with my invention. A portion of the ingot is also illustrated.

The mold is indicated at M, the ingot at I, 55 its cavity at C, and the shrink head casing is indicated at F. The core, or body of the

shrink head casing, is indicated at  $\alpha$ , and its covering at  $\gamma$ . The core of the casing is composed of slowly combustible material such as charcoal, coal, or coke mixed with 60 binding material such as cement, preferably Portland cement, in the proportions by weight of 80% combustible material, and 20% binding material. The covering,  $\gamma$ , is composed of non-combustible material, preferably silica sand, and molasses, in the proportions by weight of silica sand 75%, water 65 20%, and molasses 5%.

The feeder is provided with holes  $\alpha$  which extend through the top of the covering  $\gamma$ . 70 These are vent holes for the purpose of allowing such gases as may be generated to pass out.

A shrink head casing thus constructed 75 serves to conserve the heat of the upper portion of the ingot while being cast. The molten metal remains liquid to such an extent as to cause the pipe to be filled to a level above the bottom of the casing, and the casing as a whole is strong and of relatively 80 low weight, and may be manufactured at relatively low cost.

In the manufacture of my shrink head casing the core  $\alpha$  is first molded in any usual way, and when cold is dipped into a bath 85 composed of silica sand (silica flour), molasses and water, in the proportions above specified. The bath has the consistency of thick molasses and it is heated to a temperature preferably of about 150° F. The core 90  $\alpha$  when cold is dipped into this bath and receives a coating  $\gamma$  of approximately one-eighth of an inch thickness. After being thus dipped and after having received said coating, the casing as a whole is baked at a temperature above the boiling point of water, 95 preferably at a temperature of 250° F., until it is thoroughly dry and hard. The coating being siliceous resembles glass, and it is extremely hard and strong.

It will be observed that the combustible material  $\alpha$  does not come into direct contact with the molten metal of the ingot, and that no gas from the combustible material can pass through the coating to the ingot. My 105 shrink head casing therefore has an advantage over some feeders or shrink head casings heretofore employed.

Inasmuch as the coating  $\gamma$  is non-combustible and is of substantial thickness and 110 strength and inasmuch as its melting point is below that of liquid steel, the casing as a

whole will retain its shape until the ingot is formed, and it may then be removed from the mold with the ingot and separated therefrom with the crop end of the ingot in the 5 usual way.

I claim as my invention:

1. A shrink head casing for ingot molds comprising a self-supporting core consisting of slowly combustible material and a non- 10 metallic self-supporting casing, which completely surrounds the core, composed of non-combustible material, but having vent holes at its upper end.

2. A shrink head casing for ingot molds 15 comprising a self-supporting core consisting

of a slowly combustible material and a binder, and a covering therefor consisting of siliceous material which completely surrounds the core having only vent holes at its upper end.

3. A shrink head casing for ingot molds comprising a self-supporting core composed of slowly combustible material and a binder and a covering therefor consisting of silica sand and a binder which completely surrounds the core, but having vent holes at the top for the escape of gases.

In testimony whereof, I have hereunto subscribed my name.

EMIL GATHMANN.